

# UNITED STATES PATENT OFFICE.

ROYER LUCKENBACH, OF BROOKLYN, NEW YORK, ASSIGNOR TO LUCKENBACH PROCESSES, INC., OF SAN FRANCISCO, CALIFORNIA, A CORPORATION OF NEVADA.

## FLOTATION PROCESS.

1,425,327.

Specification of Letters Patent. Patented Aug. 8, 1922.

No Drawing.

Application filed February 9, 1920. Serial No. 357,355.

To all whom it may concern:

Be it known that I, ROYER LUCKENBACH, a citizen of the United States, and a resident of the borough of Brooklyn, county of 5 Kings, city and State of New York, have invented a certain new and useful Flotation Process, of which the following is a specification.

The invention relates to a reagent for use 10 in ore concentration by flotation, and to the process of using the same, and has for its objects the production of a powerful frothing and gathering agent which will be cheap to produce, economical of use, and in the 15 manufacture of which by products of considerable value in flotation will be produced.

These and further objects will more fully appear in the following specification and 20 claims.

It has been discovered that certain products of the destructive distillation, or of steam distillation of greasewood, a prickly, evergreen shrub indigenous to arid regions 25 of the United States, and possibly elsewhere, possess the quality of producing bubbles when introduced into an ore pulp and the mixture is aerated either by agitation or otherwise, and that such bubbles have a 30 strong affinity for certain minerals and mineral compounds, which will become attached to the bubbles and float therewith to the surface of the pulp and form a thick, heavy and stable froth which may be removed from the 35 surface of the pulp with the attached mineral values, leaving the valueless gangue within the pulp.

The principal products of the destructive distillation of greasewood comprise gas, a 40 watery liquid, a thick, pasty semi liquid, resembling in appearance coal tar, and charcoal. The thick, pasty mass, which for the purposes of this application may be termed "greasetar," although the product is neither 45 a grease or a tar as far as is known, is the reagent employed in carrying out the flotation process.

The greasetar in the condition in which it comes from the still may be employed in the 50 pulp, in which case it must be beaten into the water before the ore pulp is formed, or be carried through the pulverizing apparatus with the ore before the formation of the pulp to break it up into minute globules.

5 The preferred method, however, is to so

treat the greasetar that it will be rendered miscible in water before it is introduced into the water. By this method of treating the reagent it may be placed in the pulp in the apparatus in which flotation is effected and 60 the cost of the preliminary water treatment will be avoided. Any material which will so cut the greasetar as to make it capable of thorough mixing with the water of the pulp may be employed. It has been found that 65 alcohol or alcoholic alkali, or alkaline acetone is suitable for this purpose.

The pasty semiliquid distillate resulting from the steam distillation of the various varieties of greasewood common to the arid 70 regions of the west, and which differs somewhat in appearance, at least, from the product of destructive distillation of the greasetar is also a valuable frothing and gathering agent, and applicant does not desire to limit 75 himself to the product of destructive distillation alone, but the product of steam distillation may be used in approximately the same proportions, and the term "greasetar" used herein is intended to describe the product of either steam or destructive distillation.

In compounding the reagent formed by the destructive distillation of greasewood, 10 cc. of the greasetar distillate is dissolved in 80 approximately 15 cc. of alcoholic potash, and the solution is diluted with about 1 liter of water, to form a stock solution. In use stock 85 solution of the strength given is added to the pulp in about the proportion of 5 cc. of 90 stock solution to about 15 liters of pulp water.

No hard and fast rule as to the proportion of stock solution to the pulp water, or on the ore can be given as different ores and 95 different grades of the same ore will require different treatment. The stock solution may be added to the pulp in small quantities until the appearance of the froth produced indicates to the mill man that a proper concentration 100 is being floated.

The alcohol and alkali in the stock solution will increase the frothing properties of the mixture, and the alkali will act to sharpen the separation between the concentrate and gangue, thus taking advantage 105 of the well known effect of alkalies upon the flotation of various ores.

The alcoholic potash, when used, is preferably a 10% solution of KOH in alcohol. 110

Instead of potash, caustic soda in the same proportions may be employed. Instead of the alcohol solution of potash or soda, a 10% solution of a similar alkali in acetone, or a mixture of alcohol and acetone solutions may be employed.

A sample of 50 grams of ore from the Gogama mines of Canada, containing 7.4% of Cu. was treated in a Ruth flotation machine for 10 minutes with the stock solution as first above given. The concentrate weighed 13.3 grams and assayed 18.85% Cu. The tails weighed 30.5 grams with a copper content of 2.4%. The result showed an extraction of 77.5% of the mineral content of the ore.

A sample of 50 grams of the same was treated in the same manner and with a reagent containing 10 grams of the product of steam distillation of grease-wood instead of the greasetar, and an extraction of 91% was secured.

In the distillation of the greasewood the entire plant, including root, trunk, branches and leaves is used.

The alcohol employed may be ethyl, methyl or denatured.

While the greasetar is particularly applicable for use as a frothing and gathering reagent in ore flotation, it may be employed for other purpose such as a disinfectant for example.

In accordance with the provisions of the patent statutes I have described the principle of my invention, together with the apparatus which I now consider to represent the best embodiment thereof, but I desire to have it understood that the apparatus shown is merely illustrative, and that the invention may be carried out in other ways.

Having thus described my invention what I claim as new and desire to secure by Letters Patent, is:—

1. The process of concentrating ore by flotation, which comprises adding greasetar product of the distillation of greasewood to the pulp, aerating the pulp to form a froth, and separating the froth from the pulp. 45

2. The process of concentrating ore by flotation, which comprises adding a reagent 50 comprising the reaction product of the greasetar distillate of greasewood and an alkali, and alcohol to the pulp, aerating the pulp to form a froth and separating the froth from the pulp.

3. The process of concentrating ore by flotation, which comprises adding a reagent comprising the reaction product of the greasetar distillate of greasewood and an alkali, and alcohol and acetone to the pulp, 60 aerating the pulp to form a froth and separating the froth from the pulp.

4. The process of concentrating ore by flotation, which comprises adding the greasetar product of the distillation of 65 greasewood and alcohol to the pulp, aerating the pulp to form a froth, and separating the froth from the pulp.

5. The process of concentrating ore by flotation, which comprises adding the 70 greasetar product of the distillation of greasewood and alcohol and acetone to the pulp, aerating the pulp to form a froth, and separating the froth from the pulp.

This specification signed and witnessed 75 this sixth day of February, 1920.

ROYER LUCKENBACH.

Witnesses:

A. E. RENTON,  
H. LE BERTHON,